

# United States Patent [19]

Werneke

[11] 3,785,488

[45] Jan. 15, 1974

[54] FLOTATION PROCESS FOR RECOVERING MOLYBDENUM

[75] Inventor: Michael Francis Werneke, Milford, Conn.

[73] Assignee: American Cyanamid Company, Stamford, Conn.

[22] Filed: Apr. 27, 1972

[21] Appl. No.: 248,317

[52] U.S. Cl. .... 209/167

[51] Int. Cl. .... B03d 1/06

[58] Field of Search..... 209/166, 167

## [56] References Cited

### UNITED STATES PATENTS

1,839,155 12/1931 Lubs ..... 209/166  
1,904,460 4/1933 Moses ..... 209/166

|           |        |              |         |
|-----------|--------|--------------|---------|
| 2,125,337 | 8/1938 | Gaudin ..... | 209/166 |
| 2,316,743 | 4/1943 | Marsh .....  | 209/166 |
| 3,405,581 | 8/1946 | Keller ..... | 209/166 |

### FOREIGN PATENTS OR APPLICATIONS

114,078 10/1941 Australia..... 209/166

Primary Examiner—Robert Halper

Attorney—John M. Miele

## [57] ABSTRACT

A process for recovering molybdenite from a metallurgical concentrate comprising a major proportion of copper sulfide and other sulfides and a minor portion of molybdenum sulfide is provided, in which the copper and other sulfides are selectively depressed by employing a mixed thiol-alcohol thereby enabling the molybdenite to be recovered by flotation.

3 Claims, No Drawings

## FLOTATION PROCESS FOR RECOVERING MOLYBDENUM

Generally stated, the subject matter of the present invention relates to an improved flotation process for recovering molybdenite. More particularly, this invention relates to a process wherein molybdenum sulfide is separated from other sulfides with which it occurs by use of a novel selective depressant.

### BACKGROUND OF THE INVENTION

In the treatment of copper sulfide ores containing minor quantities of molybdenite ( $MoS_2$ ) the molybdenite normally accompanies the copper sulfide in the metallurgical concentrates obtained by flotation treatment of the raw ores. It is then necessary to separate molybdenite from the copper sulfide and any other sulfides, notably iron sulfide, in the concentrates thus obtained.

Normally, any one of three approaches may be used to separate molybdenite from other sulfides. In a first approach, molybdenite can be depressed by suitable reagents and the copper recovered by refloating. A heat treatment step involving low temperature roasting of the molybdenite bearing flotation tailings is required in order to reactivate the molybdenite for up-grading by refloating in several stages. This approach is not particularly desirable because it requires floating the major portion (usually more than 99 percent) of the metallurgical concentrate initially obtained and requires costly heat treatment as an added step.

A second approach involves depressing copper minerals by means of steaming or low temperature roasting to remove the original copper mineral collectors, followed by flotation of molybdenite from the heat treated concentrate with or without the use of auxiliary copper depressants. This approach is not particularly desirable because of the added costly heat treatment steps required.

A third approach is that of depressing copper sulfide with selective reagents and recovering molybdenite by selective flotation and repeated cleaning, as necessary. This approach is highly desirable since it requires floating only a small fraction of the total weight of metallurgical concentrate (usually less than 1 percent) and it does not require the added costly, heat treating steps. The major problem associated with this third approach is providing selective and effective depressants for sulfides other than molybdenite.

In the past, a selective depressant employed was the material obtained by reaction of sodium hydroxide with phosphorus pentasulfide commonly referred to as Noke's Reagent. This reaction may erupt with great violence liberating substantial amounts of hydrogen sulfide, a hazardous and toxic pollutant. The reaction is spasmodic in character, giving rise to violent bursts of activity and gas liberation at unpredictable intervals. The unpredictable nature of the reaction recently was responsible for the deaths of several workers. Thus, although this third approach as a method of recovering molybdenite from other sulfides is highly desirable from a processing viewpoint, the lack of safe and effective depressants necessitates the use of alternative recovery procedures. Other depressants which have been used are sodium sulfide and sodium cyanide among others. However, the sodium sulfide requires the use of large quantities, as well as constituting a safety hazard

in that it will liberate hydrogen sulfide under certain conditions. The sodium cyanide also presents a potential safety hazard because of the inherent nature of cyanide compounds.

The present invention represents the culmination of a long series of investigations directed to providing a safe and effective process for recovering molybdenite from the metallurgical concentrates obtained by the flotation treatment of raw copper sulfide ores.

Accordingly, it is an object of the invention to provide a process for recovering molybdenite from the metallurgical concentrates in which it occurs.

An additional object of the invention is to provide a safe and effective process for recovering molybdenite.

It is yet another object of the invention to provide a relatively cheap process for recovering molybdenite.

Additional objects and advantages will be set forth in part in the description which follows and in part will be obvious from the description or may be learned by the practice of the invention, the objects and advantages being realized and attained by means of the processes and improvements, particularly pointed out in the appended claims.

### THE INVENTION

To achieve the foregoing objects and in accordance with its purposes as embodied and broadly described, the present invention provides a process for recovering molybdenite from a metallurgical concentrate of sulfide minerals in which the molybdenite constitutes a minor amount which comprises depressing minerals other than molybdenite with from about 0.1 to 10 pounds per ton of concentrate of a thioalcohol having the formula:



wherein R is an alkyl group of from 1 to 4 carbon atoms, R', R'' and R''' are individually selected from hydrogen, hydroxyl, sulfhydryl and an alkanol group of from 1 to 4 carbon atoms and X is selected from hydrogen, sodium, potassium and ammonium; selectively froth floating molybdenite from the depressed sulfides and recovering the flotation concentrate thus obtained.

Thioglycerol,  $HSCH_2CH(OH)CH_2OH$ , is preferred as a selective depressant for the sulfide minerals, other than molybdenite, which have been previously activated by flotation collectors such as xanthates, dithiophosphates, dithiocarbamates and their derivatives.

The invention consists of the novel methods, processes, steps and improvements herein shown and described.

It is to be understood that both the foregoing general description and the following detailed description are exemplary and explanatory and are not restrictive of the invention.

In accordance with the present invention, the novel depressants selectively depress sulfide minerals other than molybdenite enabling much cleaner froth flotation concentrates to be obtained than was formerly possible. In addition, the present process avoids costly added heat treatment steps and enables the desired recovery to be effected while froth floating only a minor portion of the metallurgical concentrate initially em-

ployed. In addition, the reagents are safe to use and present no significant threat to health and the environment. Still further, the present process enables more efficient recovery of molybdenite to be achieved than was previously possible.

While it is not considered to limit the invention herein disclosed and claimed, it is believed that the mechanism of action involves the choice of a selective reactive moiety which has an affinity for the mineral to be depressed and attaching a hydrophilic group to such reactive moiety. Therefore, on flotation the surface of the depressed mineral has been made hydrophilic and is rendered unfloatable.

It is conceivable that the reagents used in this invention may function generally as depressants for many sulfide minerals and could be useful for example for depressing pyrite in coal flotation, to give low sulfur coal, a commodity much in demand for ecological reasons. It is also possible that they may serve to depress undesirable sulfides during non-metallic mineral flotation, for example, in the recovery of fluorspar, barite, silica, feldspar, etc., from their ores.

Applications of other materials as depressants could include the use of hydrophilic polycarboxylic acids or sulfonates to depress minerals which are normally promoted by fatty acids or petroleum sulfonates. Hydrophilic polyamines may be used as depressants for minerals which are promoted by fatty amines.

In carrying out the process of the present invention, a copper ore in which the metal occurs as a sulfide is first processed in accordance with conventional procedures to separate the valuable minerals from the gangue materials. Generally, such separation is effected by grinding the ore to a suitable size for flotation and effecting flotation using a collector such as a xanthate, dithiophosphate, dithiocarbamate, or a derivative thereof. The concentrate thus collected is suitable for use directly in the process of the present invention. The particular method by which the metallurgical concentrate is obtained is not critical and forms no part of the present invention.

The metallurgical concentrate is prepared as a 15-40 percent aqueous slurry in a flotation cell and conditioned with from about 0.1 to about 10 pounds per ton of solids with a novel depressant of the present invention. The most effective amount can be readily determined by testing. Conditioning is continued until copper sulfide is no longer floated to the surface by a stream of air. The use of a hydrocarbon oil in sufficient amount to aid in the flotation of the molybdenum sulfide to the surface where it can be collected is also possible. Hydrocarbon oils such as kerosene, fuel oil, and the like are normally used for such purpose and are effective in the present process.

The floated molybdenum sulfide concentrate is then recovered and, if necessary, subjected to cleaning. In many instances the concentrate obtained is of sufficient purity to be processed without the need for additional cleaning. When cleaning is contemplated, a re flotation of the concentrate using a novel depressant of the present invention is beneficial.

The following examples are provided for illustrative purposes and may include particular features of the invention. However, the examples should not be construed as limiting the invention, many variations of which are possible without departing from the spirit or scope thereof.

#### EXAMPLE I

A 600 gm. sample of mixed copper-molybdenum sulfides containing ~0.55 percent molybdenum was re-floated in a laboratory flotation cell at ~28 percent solids with 0.1 lb./ton of sodium ethyl xanthate for 5 minutes. The froth product was returned to the cell, conditioned for 2 minutes with 2.00 lbs./ton of thioglycerol, HSCH<sub>2</sub>CH(OH)CH<sub>2</sub>OH, and 0.5 lb./ton of fuel oil. The froth was collected for 4 minutes, returned to a cleaner cell, conditioned for 2 minutes with 0.5 lb./ton of thioglycerol and 0.2 lb./ton fuel oil and the froth collected for 4 minutes more. The cleaned concentrate contained 9.2 percent of the total sample weight, while the rougher tailing contained 71.8 percent and the cleaner tailing 19.0 percent. Microscopic examination showed that >95 percent of the molybdenum had been recovered in the rougher flotation step.

#### EXAMPLE II

A copper concentrate was processed in the laboratory using thioglycerol to depress the copper minerals while recovering the contained molybdenum minerals by froth flotation. The following operating procedure was employed:

##### 9CTA

| Operation   | Minutes | % Solids | pH      | Reagents9CTA<br>(lbs./ton feed)9CTA<br>Thio- Fuel9CTA<br>glyc- Oil9CTA<br>erol9CTA |
|-------------|---------|----------|---------|------------------------------------------------------------------------------------|
| Condition   | 1.5     | 30       |         | 1.0 0.29CTA                                                                        |
| Rougher9CTA |         |          |         |                                                                                    |
| Flotation   | 8.0     | 30       | 9.59CTA |                                                                                    |
| Rougher9CTA |         |          |         |                                                                                    |
| Flotation   | 6.0     | 30       |         | 0.259CTA                                                                           |
| Cleaner9CTA |         |          |         |                                                                                    |
| Flotation   | 3.0     | 20       |         | 0.50                                                                               |

The following metallurgical results were obtained:

| Product     | Wgt. % | % Mo  | Assay9CTL % Cu | Distribution9CTA<br>% Mo% Cu9CTA |
|-------------|--------|-------|----------------|----------------------------------|
| Rougher9CTA |        |       |                |                                  |
| Tailing     | 88.06  | 0.153 | 49.5           | 15.2887.819CTA                   |
| Cleaner9CTA |        |       |                |                                  |
| Tailing     | 4.94   | 0.990 | 52.5           | 5.55 5.229CTA                    |
| Cleaner9CTA |        |       |                |                                  |
| Conc.       | 7.00   | 9.970 | 49.5           | 79.17 6.979CTA                   |
| Calc. Feed  | 100.0  | 0.88  | 49.6           | 100.0 100.0                      |

#### EXAMPLE III

Comparison of current plant operating practice with Noke's Reagent relative to thioglycerol for copper depression during rougher molybdenum flotation is as follows:

##### 9CTA

| Example | Reagent      | Concentration9CTL<br>lbs./ton9CTL | Percent 9CTA<br>Copper9CTA<br>depression9CTA |
|---------|--------------|-----------------------------------|----------------------------------------------|
| 9CTL    | —            | —9CTL                             | 21.39CTA                                     |
| I-a     | —            | 29CTL                             | 46.09CTA                                     |
| I-b     | Noke's rgt.  | 49CTL                             | 75.09CTA                                     |
| I-c     | Noke's rgt.  | 19CTL                             | 87.89CTA                                     |
| I-d     | Thioglycerol | 49CTL                             | 94.6                                         |
| I-e     | Thioglycerol |                                   |                                              |

It can be readily observed from the examples that the reagents of this invention are extremely effective at depressing the copper sulfide minerals, while allowing the molybdenum sulfide to float and be concentrated.

I claim:

1. A process for recovering molybdenite from a metallurgical concentrate which comprises depressing sulfide minerals other than molybdenite with from about 0.1 to 10 pounds per ton of concentrate solids of thioglycerol, selectively froth-floating molybdenite from

the sulfides and recovering the flotation concentrate thus obtained.

2. A process according to claim 1 wherein the concentration of the thioglycerol is from about 1 to 4 pounds per ton.

5

10

15

20

25

30

35

40

45

50

55

60

65

3. A process according to claim 1 wherein a hydrocarbon oil is used to aid in the flotation and recovery of the molybdenite.

\* \* \* \* \*